

## 1

2,903,325

PROCESS FOR PRODUCING OR STRIPPING  
DYEINGSWilhelm Geigy, Binningen, Switzerland, assignor to Ciba  
Limited, Basel, Switzerland, a Swiss firmNo Drawing. Application May 13, 1957  
Serial No. 658,527Claims priority, application Switzerland  
January 29, 1954

8 Claims. (Cl. 8—43)

This application is a continuation-in-part of my co-pending application Serial No. 484,057, filed January 25, 1955 (and abandoned since the filing of the present application).

This invention is based on the observation that polyvinyl-pyrrolidone, if desired, in conjunction with another ion-free agent, is a good levelling agent or stripping agent in the production or stripping of dyeings on nitrogenous basic fibrous materials of complex metal compounds, especially chromium or cobalt compounds, of monoazo-dyestuffs free from sulfonic acid groups and containing less than one atomic proportion of metal bound in complex union per molecular proportion of monoazo-dyestuff.

For the purposes of the present invention ordinary commercial polyvinyl-pyrrolidone may be used. There are suitable e.g. polyvinyl-pyrrolidones having a molecular weight ranging from 5000 to 50,000 (average 25,000), those having a molecular weight ranging from 20,000 to 80,000 (average 50,000) or those having an average molecular weight of 700,000. As ion-free agents which may, if desired, be used in conjunction with the polyvinyl-pyrrolidone there come into consideration more especially ethylene oxide condensation products of fatty alcohols, of fatty amines or of alkyl-phenols. There may be mentioned, for example, the condensation product of 1 molecular proportion of para-tertiary-octyl-phenol with about 8 molecular proportions of ethylene oxide or the condensation product of 1 molecular proportion of octadecyl alcohol with about 25 molecular proportions of ethylene oxide, and also the condensation product of 1 molecular proportion of oleylamine with about 12 molecular proportions of ethylene oxide. The relative proportions of the polyvinyl-pyrrolidone and the other ion-free agent may vary within wide limits, but there are advantageously used mixtures of which at least one half consists of polyvinyl-pyrrolidone.

The dyeing with a complex metal compound of the kind described above, of which a large number is known in the literature, is carried out in the usual manner. The levelling agent may simply be added to the dyebath. The proportion in which it is added usually amounts to a few parts per mil on the weight of the fibrous material.

The stripping of a dyeing by the process of the invention is advantageously carried out at a raised temperature, for example, at the boiling temperature. For this purpose it usually suffices to use a few parts percent of the stripping agent calculated on the weight of the fibrous material. If desired, a reducing compound, such as a hydrosulfite, may also be added.

As nitrogenous basic fibrous materials, on which a dyeing may be produced or from which a dyeing may be stripped, there come into consideration more especially wool, and also silk or synthetic fibers having similar properties obtained from casein or polyamide or polyurethane fibers. There may also be used mixtures of basic fibers with other fibers, for example, nitrogenous non-basic fibers, such as polyacrylonitrile fibers, and also

## 2

fibers of polyvinyl chloride or polyester fibers. The fibrous material may be treated in loose condition or in the form of a yarn, hank or fabric, or in the form of foil. The present process is especially suitable for the treatment of wool.

The following examples illustrate the invention, the parts being by weight unless otherwise stated and the relationship of parts by weight to parts by volume being the same as that of the kilogram to the liter.

## Example 1

Wool is dyed at the boiling temperature in a dyebath, which has been adjusted with sodium phosphate to a pH value of 6.5 and contains 0.25% of the bordeaux dyeing cobalt complex of the dyestuff of the formula



and 0.25% of a mixture of equal parts of polyvinyl-pyrrolidone and the condensation product of one molecular proportion of commercial octadecyl alcohol with about 25 molecular proportions of ethylene oxide. (The percentages are calculated on the weight of the fibrous material). The dyeing is then finished in the usual manner. There is obtained a substantially more level dyeing than is obtained without the addition of the levelling agent.

In the same manner the yellowish red dyeing chromium 1:2 complex of the dyestuff of the formula



can be used to produce more level dyeings.

Similar results are obtained by using polyvinyl-pyrrolidone alone, instead of the aforesaid mixture.

## Example 2

In order to strip a dyeing the procedure may be as follows: Wool, which has been dyed with 1% of the reddish blue dyeing chromium complex of the dyestuff of the formula



is treated for one hour at the boiling temperature and at a liquor ratio of 1:40 in a bath which contains 4% of polyvinyl-pyrrolidone calculated on the weight of the fibrous material. The material is then rinsed and dried. The dyestuff is stripped to a considerable extent in this manner.

A smaller quantity of polyvinyl-pyrrolidone may be used, for example, 1 or 2%, and in this manner the dyeing is rendered considerably lighter.

Instead of using polyvinyl-pyrrolidone alone, there may be used the mixture described in Example 1 or a mixture

of polyvinyl-pyrrolidone and a condensation product of 1-molecular proportion of oleylamine and 10-14-molecular proportions of ethylene oxide.

*Example 3*

A wool fabric is dyed at the boiling temperature in a dyebath which has been adjusted with ammonium acetate to a pH value of 6.3 and contains 0.25% of the red dyeing cobalt 1:2 complex of the dyestuff of the formula



and 0.2% of a polyvinyl-pyrrolidone having an average molecular weight 40,000. (The percentages are calculated on the weight of the fibrous material.) The dyeing is then finished in the usual manner. There is obtained a substantially more level dyeing than is obtained without the addition of the levelling agent.

In the same manner the following metal complexes of monoazo-dyestuffs can be used to produce more level dyeings:

The grey-blue dyeing cobalt 1:2 complex or the violet dyeing chromium 1:2 complex of the dyestuff of the formula



The red dyeing cobalt 1:2 complex of the dyestuff of the formula



The steel-blue dyeing chromium 1:2 complex of the dyestuff of the formula



Similar results are obtained by using a polyvinyl-pyrrolidone having an average molecular weight of 700,000 instead of a polyvinyl-pyrrolidone having an average molecular weight of 40,000.

*Example 4*

A wool fabric is dyed at the boiling temperature in a dyebath which has been adjusted with ammonium acetate to a pH value of 6.3 and contains 0.25% of the brown

7  
dyeing chromium 1:2 complex of the dyestuff of the formula



10 and 0.2% of a polyvinyl-pyrrolidone having an average molecular weight 40,000. (The percentages are calculated on the weight of the fibrous material.) The dyeing is then finished in the usual manner. There is obtained a substantially more level dyeing than is obtained without the addition of the levelling agent.

15 In the same manner, the brownish red dyeing cobalt 1:2 complex of the formula



20 can be used to produce more level dyeings.

25 Similar results are obtained by using a polyvinyl-pyrrolidone having an average molecular weight of 700,000 instead of a polyvinyl-pyrrolidone having an average molecular weight of 40,000.

*Example 5*

30 A wool fabric is dyed at the boiling temperature in a dyebath which has been adjusted with ammonium acetate to a pH value of 6.3 and contains 0.25% of the green dyeing cobalt 1:2 complex of the dyestuff of the formula



35 and 0.2% of a polyvinyl-pyrrolidone having an average molecular weight of 700,000. (The percentages are calculated on the weight of the fibrous material.) The dyeing is then finished in the usual manner. There is obtained a substantially more level dyeing than is obtained without the addition of the levelling agent.

40 In the same manner the following metal complexes of monoazo-dyestuffs can be used to produce more level dyeings:

45 The lilac dyeing chromium 1:2 complex of the dyestuff of the formula



50 55 60 65 70 75 The green dyeing chromium 1:2 complex or the greyish-violet dyeing cobalt 1:2 complex of the dyestuff of the formula



The greyish green dyeing chromium 1:2 complex of the dyestuff of the formula



And the steel-blue dyeing chromium 1:2 complex of the dyestuff of the formula



Similar results are obtained by using a polyvinyl-pyrrolidone having an average molecular weight of 40,000 instead of a polyvinyl-pyrrolidone having an average molecular weight of 700,000.

What is claimed is:

1. In the process of shifting the distribution equilibrium, between an aqueous dye bath and wool, of a complex metal compound of a monoazo dyestuff which is free from sulfonic acid groups



and contains less than one atomic proportion of a metal selected from the group consisting of cobalt and chromium bound in complex union per molecular proportion of dyestuff, the improvement of simultaneously incorporating into said aqueous bath polyvinyl-pyrrolidone, in addition to said wool and said complex metal compound.

2. In the process of shifting the distribution equilibrium, between an aqueous dye bath and wool, of a complex metal compound of an ortho,ortho'-dihydroxy-mono-azo dyestuff which is free from sulfonic acid groups



and contains less than one atomic proportion of a metal selected from the group consisting of cobalt and chromium bound in complex union per molecular proportion of dyestuff, the improvement of simultaneously incorporating into said aqueous bath polyvinyl-pyrrolidone, in addition to said wool and said complex metal compound.

3. In the process of shifting the distribution equilibrium, between an aqueous dye bath and wool, of a complex metal compound of an ortho,ortho'-dihydroxy mono-azo dyestuff which is free from sulfonic acid groups



and contains less than one atomic proportion of a metal selected from the group consisting of cobalt and chromium bound in complex union per molecular proportion of dyestuff and which further contains at least one sulfonamide group in an aromatic nucleus, the improvement of simultaneously incorporating into said aqueous bath polyvinyl-pyrrolidone, in addition to said wool and said complex metal compound.

4. In the process of shifting the distribution equilibrium, between an aqueous dye bath and wool, of a com-

plex metal compound of an ortho,ortho'-dihydroxy mono-azo dyestuff which is free from sulfonic acid groups



and contains less than one atomic proportion of a metal selected from the group consisting of cobalt and chromium bound in complex union per molecular proportion of dyestuff and which further contains at least one sulfonamide group in an aromatic nucleus, the improvement of simultaneously incorporating into said aqueous bath polyvinyl-pyrrolidone and a condensation product of a fatty alcohol with ethylene oxide, in addition to said wool and said complex metal compound.

5. In the process of shifting the distribution equilibrium, between an aqueous dye bath and wool, of a complex metal compound of an ortho,ortho'-dihydroxy mono-azo dyestuff which is free from sulfonic acid groups



25 and contains less than one atomic proportion of a metal selected from the group consisting of cobalt and chromium bound in complex union per molecular proportion of dyestuff and which further contains at least one sulfonamide group in an aromatic nucleus, the improvement of simultaneously incorporating into said aqueous bath polyvinylpyrrolidone and the condensation product of 1 molecular proportion of octadecyl alcohol with about 25 molecular proportions of ethylene oxide, in addition to said wool and said complex metal compound.

35 6. In the process of shifting the distribution equilibrium, between an aqueous dye bath and wool, of a complex chromium compound of an ortho,ortho'-dihydroxy mono-azo dyestuff which is free from sulfonic acid groups



40 and contains less than one atomic proportion of chromium bound in complex union per molecular proportion of dyestuff and which further contains at least one sulfonamide group in an aromatic nucleus, the improvement of simultaneously incorporating into said aqueous bath polyvinyl-pyrrolidone, in addition to said wool and said complex chromium compound.

55 7. In the process of shifting the distribution equilibrium, between an aqueous dye bath and wool, of a complex cobalt compound of an ortho,ortho'-dihydroxy mono-azo dyestuff which is free from sulfonic acid groups



60 and contains less than one atomic proportion of cobalt bound in complex union per molecular proportion of dyestuff and which further contains at least one sulfonamide group in an aromatic nucleus, the improvement of simultaneously incorporating into said aqueous bath polyvinyl-pyrrolidone, in addition to said wool and said complex cobalt compound.

70 8. In the process of shifting the distribution equilibrium, between an aqueous dye bath and wool, of a complex metal compound of an ortho,ortho'-dihydroxy mono-azo dyestuff which is free from sulfonic acid groups



75 and contains less than one atomic proportion of a metal

selected from the group consisting of cobalt and chromium bound in complex union per molecular proportion of dyestuff and which further contains at least one sulfamide group in an aromatic nucleus, the improvement of simultaneously incorporating into said aqueous bath a polyvinyl-pyrrolidone and the condensation product of 1 molecular proportion of oleylamine with 10 to 14 molec-

8  
ular proportions of ethylene oxide, in addition to said wool and said complex metal compound.

References Cited in the file of this patent

Melliand, XXXII, for January 1951, pp. 53-56.  
American Dyestuff Reporter for Feb. 1, 1954, pp. 72-75.